

# United States Patent Office

3,051,655

Patented Aug. 28, 1962

1

3,051,655

## METALWORKING LUBRICANT

George E. Barker, Norristown, Pa., assignor to Quaker Chemical Products Corporation, Conshohocken, Pa., a corporation of Pennsylvania  
No Drawing. Filed Nov. 1, 1957, Ser. No. 693,808  
1 Claim. (Cl. 252—49.9)

This invention relates to lubricants for the lubrication of metals under conditions of working such as rolling, drawing, extruding, cutting, grinding, forging and spinning.

It is customary to use a variety of lubricants for metalworking depending on the operation and the requirements of the job. A particular characteristic of metalworking operations is the existence of high unit pressures. Consequently, the lubricant must maintain its lubrication under these boundary conditions. For most metalworking activities the surface friction must be low in order to prevent contributing to the heat generated by the metal deformation and to reduce the pressure necessary to obtain the desired degree of deformation such as in rolling or drawing. Under some conditions physical dissipation of heat, e.g., by water cooling, is required, and the lubricant should interfere with this cooling to a very minimum extent.

It is well known that fatty oils and fatty acids are widely used as metalworking lubricants because of their friction-reducing properties under high pressures, e.g., the use of palm oil in cold rolling steel. These boundary lubricating properties of the fatty oils involve physical and chemical adsorption of their polar constituents. There is much evidence that the long chain polar compounds in fats orient themselves at the surface and thus aid in maintaining low friction under high pressures. However, fatty oils have several disadvantages including gumming, carbonizing, becoming rancid and having variable compositions. They also are subject to a fluctuating price structure, and some of the most useful fats such as palm oil are subject to scarcity during times of political unrest in many sections of the world.

It is an object of this invention to produce a new and superior metalworking lubricant. It is also an object of this invention to produce metalworking lubricants which obviate the use of fatty oils, or reduce the proportion of fatty oils required for a given metal working operation. Another object of this invention is to produce lubricants superior to fatty oils. A corollary object of this invention is to produce a metalworking lubricant which will not gum, carbonize or otherwise decompose to produce a contaminated metal surface difficult to clean. Compositions of this invention leave essentially no residue after annealing of metal which has been stamped, drawn or rolled.

In accordance with this invention it has been found that a new and useful family of metalworking compounds may be prepared by reacting long chain amines with phosphoric acid. According to my invention, I use those amines containing at least one carbon chain possessing from 12 to 30 carbon atoms. They preferably are di- or polyfunctional amines and may be primary, secondary or tertiary or a mixture of the three.

I believe these compounds may be generically represented by the following structural formula:



where R is an alkyl group containing at least one carbon chain possessing from 12 to 30 carbon atoms; R' is selected from H, alkyl, ethoxy, polyethoxy, aminoalkyl, or ethoxylated aminoalkyl groups; R'' is selected from H,

2

alkyl, ethoxy, or polyethoxy groups; n is 1 to 3; and m is 1 or 2.

As indicated, R' may be substituted by an amino radical which, in turn, may have one or both of its hydrogen atoms replaced by alkyl groups or ethoxy or polyethoxy groups. When R' is thus substituted by an amino group, m may be any value up to and including 2, whereby compounds of the following structural formula are produced:



where x is an integer of 1 to 3.

I believe the compounds of this invention are the primary or secondary phosphate salts of the amines or mixtures of the two, (n=1 or 2) since it has been reported in the literature (Hoerr and Ralston, J.A.C.S. 64, 2824 (1942) that attempts to isolate the tertiary phosphates of long chain aliphatic amines have been unsuccessful. However, I do not wish to limit the invention by this statement, particularly in view of the fact that I obtain excellent metalworking lubricants, when using the amines even in excess of the 3 amino groups per mol of phosphoric acid as indicated above.

Because of the ready dispersibility in diluents such as mineral oil or water, oxyethylated derivatives of the above described amines such as those in which these amines are condensed with one to five mols of ethylene oxide per primary or secondary amine group are preferred. The ratio of alkylamine to phosphoric acid may vary over a wide range depending on the application of the lubricant. For example, it may be as high as 2 or 3 mols of phosphoric acid per amine group in cases where simultaneous phosphating of the steel is desirable such as in some compounds for making extremely severe draws. On the other hand it may be as low as 0.01 to 0.1 mol of phosphoric acid per amine group, where the lubricating requirements are light or moderate or an alkaline agent is desired. Naturally, for most applications 0.1 to 0.5 mol of phosphoric acid per amine group is preferred. These compositions range from viscous liquids to waxy solids depending on the components.

These metalworking lubricants are generally employed in a diluent such as mineral oil, preferably of lubricating viscosity, in amounts of from 0.5 to 50% by weight of the compounds, or in water in the interest of economy or ease of application, but they may be applied directly for severe operations. Also, these lubricants may be applied in a volatile diluent for ease of application and the diluent evaporated to leave a tenacious adherent film. Aside from their use directly as lubricants these compositions may be added to the common lubricating agents such as fats, mineral oils, synthetic lubricants, and silicones, or mixtures thereof to enhance the lubricating properties of the latter.

To these new lubricants in mineral oil there may be added the usual types of well known modifying additives such as viscosity improvers, anti-oxidants, thickeners, graphite, molybdenum disulfide, sulfurized oils, chlorine derivatives, and the like. Generally, the addition of sulfur- or chlorine-containing compounds is unnecessary because the new lubricants exhibit excellent boundary and extreme pressure lubricating properties.

The metal working lubricants of this invention are easily made by well known techniques. Generally, it is simply necessary to mix the amine with phosphoric acid. The compositions of this invention are illustrated by the following examples.

## EXAMPLE I

28 parts of alkylaminopropylamine, where the alkyl group represents the hydrocarbon chains normally present in tallow, which fall in the approximate range of two

percent tetradecyl, 24 percent hexadecyl, 28 percent octadecyl, and 46 percent octadecenyl (available from Armour & Co. as Doumeen T or from General Mills, Inc. as Diam 26), is melted and stirred vigorously while 28.5 parts of phosphoric acid (75%) diluted with 43.5 parts of water is added slowly and stirring is continued until a smooth, uniform paste is obtained. This product is generally diluted with 3 to 10 parts of water for use. It phosphates and lubricates in one operation when the metal is treated by a suitable means such as immersion or spraying preferably with the lubricant at a temperature of 140°-180° F. This lubricant is used for drawing steel tubing as well as for the stamping, drawing or otherwise forming of metal parts.

#### EXAMPLE II

14.1 parts of an alkylamine, where the alkyl group represents the hydrocarbon chain normally present in soya oil, which falls in the approximate range of 20 percent hexadecyl, 17 percent octadecyl, 26 percent octadecenyl, and 37 percent octadecadienyl (available from Armour & Co. as Armeen S) is stirred vigorously while 6.9 parts of phosphoric acid (75%) diluted with 79.0 parts of water is added slowly until a smooth viscous fluid is obtained.

Higher amines such as those derived from behenic, arachidic and erucic acids, and the acids obtainable from beeswax and carnauba wax are also suitable for preparing these lubricants. These amines may contain up to 30 carbon atoms.

#### EXAMPLE III

7.1 parts of a tertiary alkylamine condensed with 5 mols of ethylene oxide, where the alkyl group represents an aliphatic highly branched chain hydrocarbon containing 18 to 24 carbon atoms and in which the amine group is attached to a tertiary carbon atom of the chain (available from Rohm & Haas Co. as Priminox 10) and 2.3 parts of an alkylaminopropylamine; where the alkyl group represents the hydrocarbon chain normally present in tallow (available from Armour & Co. as Duomeen T or from General Mills, Inc. as Diam 26) are melted together and stirred vigorously while 4 parts of monosodium phosphate dissolved in 86.6 parts of water is added slowly with stirring. A smooth, very viscous fluid, which may set to a thixotropic solid on standing, is obtained. When applied to a steel surface at a dilution of 1:5 in water at 160° F. for 3 minutes, followed by drying, a strongly adherent film is formed. The film serves as a good lubricant for drawing or spinning of the metal. Water dilutions of the lubricant are good grinding and cutting lubricants and coolants.

#### EXAMPLE IV

17.9 parts of a polyoxyethyl alkylaminopropylamine where the alkyl group represents the hydrocarbon chain normally present in tallow and the polyoxyethyl represents the reaction product with 3 mols of ethylene oxide per mol of amine (obtainable from Armour & Co. as Ethoduomeen T/13) is dissolved in 79.9 parts of naphthenic oil (200 SUS at 100° F.) at a temperature of 150° F. While stirring this mixture rapidly, 2.2 parts of phosphoric acid (75%) is added and the heating continued, raising the temperature of the reaction mixture gradually to 275° F. and maintaining until a clear liquid is obtained and foaming has ceased. The foaming is caused by the boiling out of the water introduced with the phosphoric acid. When applied to a metal surface this lubricant serves as an efficient metalworking lubricant for cutting, drawing and rolling. It is also self-emulsifying and efficient when dispersed in water. It is unaffected by water hardness.

#### EXAMPLE V

12.9 parts of a polyoxyethyl alkylaminopropylamine, where the alkyl group represents the hydrocarbon chain normally per molecule (available from Armour & Co. as Ethoduomeen T/15), 6.7 parts of an alkylaminopropyl-

amine, where the alkyl group represents the hydrocarbon chain normally present in tallow (available from Armour & Co. as Duomeen T and from General Mills, Inc. as Diam 26), 20 parts tallow, and 5 parts of a sulfurized petroleum oil containing about 2% sulfur are heated together (about 130° F.) to give a clear liquid. 5.4 parts of phosphoric acid (75%) is dissolved in 50 parts of water and the solution is added to the mixture of oils and amines with energetic stirring to form an emulsion. This product is an effective metalworking lubricant. It is useful when diluted for cutting and grinding coolants. It is applied diluted 1:5 with water to steel tubing, the water evaporated to leave tough adherent film and the tubing drawn to give an excellent uniform finish.

15

#### EXAMPLE VI

A mixture of 5.3 parts of a polyoxyethyl alkylaminopropylamine, where the alkyl group represents the hydrocarbon chain normally present in tallow (available from Armour & Co. as Ethoduomeen T/13), 0.8 part of alkylaminopropylamines, where the alkyl group represents the hydrocarbon chain normally present in tallow, 61 parts of naphthenic lubricating oil having a viscosity of 200 SUS at 100° F., 3 parts stearic acid, 26.9 parts tallow and 2.5 parts of a sulfurized mineral oil containing about 2% sulfur is heated to 150° F. to give a clear liquid. To the clear oil described above is added with vigorous stirring 0.50 part of phosphoric acid (75%) and the temperature is raised to 275° F. gradually and maintained there until clear and foaming (caused by boiling out of water) has ceased. This product is an excellent metalworking lubricant, particularly for rolling steel in a recirculating system, when diluted with 5 to 50 parts of water. It is also effective for cutting, grinding, drawing and other metalforming operations.

30

#### EXAMPLE VII

4.5 parts of a polyoxyethyl alkylaminopropylamine, where the alkyl group represents the hydrocarbon chain normally present in coconut oil and where the polyoxyethyl represents the reaction product of 3 moles of ethylene oxide per mole of amine (available from Armour & Co. as Ethoduomeen C/13), 0.8 part of alkylaminopropylamine, where the alkyl group represents the hydrocarbon chain normally present in coconut oil (available from Armour & Co. as Duomeen C and from General Mills, Inc. as Diam 21), 2.8 parts stearic acid, 2.5 parts sulfurized mineral oil containing about 2% sulfur and 89 parts of naphthenic petroleum oil having a viscosity of 1200 SUS at 100° F. are heated to 140° F. to give a clear liquid. To the above rapidly stirred mixture of amines and oils there is added 0.4 part of phosphoric acid (75%) and the temperature raised gradually to 290° F. and maintained there until a clear liquid is obtained and foaming has ceased. This is a very effective metalworking lubricant, especially for cutting, grinding and rolling.

40

#### EXAMPLE VIII

8 parts of alkylaminopropylamine, where the alkyl group represents the hydrocarbon chains normally present in tallow (available from Armour & Co. as Duomeen T or from General Mills, Inc. as Diam 26) is melted and stirred with 87.9 parts of mineral oil having a viscosity of 1200 SUS at 100° F. to give a clear liquid. To the oil solution of the amine is added with stirring 0.5 part of phosphoric acid (75%). The mixture is heated to 280° F. and stirring continued until a clear liquid is obtained. 2.8 parts of oleic acid is added to the above solution with stirring and the product is allowed to cool to room temperature. This product is a very suitable lubricant for drawing, rolling and cutting. It does not emulsify with water.

50

Employing a modification of the Bowden-Leben apparatus (Proc. Roy. Soc. 169, 371 (1939)) for measuring boundary friction in the presence of lubricated steel sliding on steel under calculated pressures of 200,000 to

400,000 lbs. per sq. in., the coefficient of friction using the lubricants of the examples of this invention were measured. These data are given in comparison with the performance of mineral oil and palm oil in Table I.

## EXAMPLE IX

45.2 parts of melissyl amine ( $C_{30}H_{61}NH_2$ ) is melted and dissolved in 200 parts of naphthenic oil (200 SUS at 100° F.) at a temperature of 180°–200° F. While stirring vigorously, 1.3 parts of phosphoric acid (75%) is added and the heating continued, raising the temperature of the reaction mixture gradually to 275° F. and maintaining at that temperature until a clear liquid is obtained and the foaming has ceased. When applied to a metal surface this lubricant serves as an efficient metalworking lubricant for cutting, drawing and rolling.

## EXAMPLE X

19.3 parts of di-alkylamine, where the alkyl groups represent the hydrocarbon chains normally present in hydrogenated tallow, which fall in the approximate range of 24 percent hexadecyl, 75 percent octadecyl, and one percent octadecenyl (available from Armour & Co. as Armeen 2HT or from General Mills, Inc. as Alamine H226) is dissolved in 78.3 parts of naphthenic petroleum oil having a viscosity of 200 SUS at 100° F. at a temperature of 180°–200° F. to give clear liquid. To the above rapidly stirred solution is added 2.4 parts of phosphoric acid (75%) and the temperature raised gradually to 285° F. and maintained there until a clear liquid is obtained and foaming has ceased. This is an effective lubricant for drawing, cutting and rolling.

## EXAMPLE XI

24.5 parts of dimethyldodecylamine (available from Distillation Products Division of Eastman Kodak Co.) is stirred vigorously while 13 parts of phosphoric acid (75%) diluted with 62.5 parts of water is added slowly and stirring is continued until a smooth, viscous fluid is obtained. This product is suitable for cutting and drawing. It may be diluted with water to an extent depending on its use.

Table I

## BOUNDARY LUBRICATING PROPERTIES OF METALWORKING LUBRICANTS

| Lubricant                                   | Conditions                          | Coef. of Friction |
|---------------------------------------------|-------------------------------------|-------------------|
| Example I.....                              | Applied as 1:5 dispersion in water. | 0.08 (wet).       |
| Example II.....                             | do.....                             | 0.11 (wet).       |
| Example III.....                            | do.....                             | 0.11 (wet).       |
| Example IV.....                             | Applied directly.....               | 0.10.             |
| Example V.....                              | do.....                             | 0.09.             |
| Example VI.....                             | do.....                             | 0.09.             |
| Example VII.....                            | do.....                             | 0.09.             |
| Example VIII.....                           | do.....                             | 0.09.             |
| Example IX.....                             | do.....                             | 0.09.             |
| Mineral Lubricating Oil, 200 SUS at 100° F. | do.....                             | 0.15.             |
| Palm Oil.....                               | do.....                             | 0.10.             |

To show the effects of carbon chain length of amine phosphate a homologous series was studied. The compositions were prepared by the procedure described in Example II, using 1 mol of phosphoric acid per molecular equivalent of amine and adjusting the water content to a constant 75%. For determining coefficients of friction of steel, the compositions were diluted with 5 parts of water and applied to the steel plate on which the steel ball slides. From the data presented in Table II, it is evident that there is sharp change in effectiveness between 10 and 12 carbon atoms in the alkyl chain.

6  
Table II

## BOUNDARY LUBRICATING PROPERTIES OF A HOMOLOGOUS SERIES OF n-PRIMARY ALKYLAMINE PHOSPHATES

| 5                               | Compound | Coef. of Friction |
|---------------------------------|----------|-------------------|
| n-Octylamine phosphate.....     |          | 0.14              |
| n-Decylamine phosphate.....     |          | 0.13              |
| n-Dodecylamine phosphate.....   |          | 0.10              |
| n-Octadecylamine phosphate..... |          | 0.09              |

In addition to showing excellent friction-reducing properties under boundary conditions, these lubricants show excellent extreme pressure properties as measured with the Falex Lubricant Tester. Some of these data are shown in Table III.

7  
Table III  
FALEX SEIZURE TESTS ON METALWORKING LUBRICANT

| 20 | Lubricant                                   | Conditions                                                            | Load at Seizure, Lbs. |
|----|---------------------------------------------|-----------------------------------------------------------------------|-----------------------|
| 25 | Example IV.....                             | Applied directly.....                                                 | >4,500                |
|    | Example IV.....                             | Applied diluted 1:7 with mineral lubricating oil, 100 SUS at 100° F.  | >4,500                |
|    | Example IV.....                             | Applied diluted 1:15 with mineral lubricating oil, 100 SUS at 100° F. | 3,250                 |
| 30 | Example V.....                              | Applied directly.....                                                 | >4,500                |
|    | Example VI.....                             | do.....                                                               | >4,500                |
|    | Palm Oil.....                               | Applied diluted 1:7 with mineral lubricating oil, 100 SUS at 100° F.  | >4,500                |
|    | Palm Oil.....                               | Applied diluted 1:15 with mineral lubricating oil, 100 SUS at 100° F. | 2,000                 |
|    | Palm Oil.....                               | Applied directly.....                                                 | 1,500                 |
| 35 | Mineral Lubricating Oil, 100 SUS at 100° F. | Applied directly.....                                                 | 1,200                 |

The compositions of this invention can be applied with excellent results to general metalworking operations such as grinding, cutting, drilling, drawing and rolling.

I claim:

As an improved metalworking lubricant, a composition consisting essentially of a mineral oil of lubricating viscosity and 0.5 to 50% by weight of a compound having the structural formula



50 where R is an alkyl group containing a carbon chain possessing from 12 to 30 carbon atoms; R' is selected from the group consisting of H, aminopropyl and ethoxylated aminopropyl groups; R'' is selected from the group consisting of H, and polyethoxy groups having 1 to 5 ethylene oxide residues; n is an integer 1 to 3; and m is an integer 1 to 2.

## References Cited in the file of this patent

## UNITED STATES PATENTS

|    |           |                  |               |
|----|-----------|------------------|---------------|
| 60 | 1,836,047 | Somerville       | Dec. 15, 1931 |
|    | 2,255,082 | Orthner et al.   | Sept. 9, 1941 |
|    | 2,664,400 | Woodstock et al. | Dec 29, 1953  |
|    | 2,736,658 | Pfohl et al.     | Feb. 28, 1956 |
| 65 | 2,798,045 | Buck et al.      | July 2, 1957  |
|    | 2,824,068 | Leland et al.    | Feb. 18, 1958 |
|    | 2,917,160 | Turinsky         | Dec. 15, 1959 |

## OTHER REFERENCES

70 "Priminox Series," Rohm and Haas Co., Phila., April 1955, page 2.  
Bastian: Metal Working Lubricants, McGraw-Hill Book Co., N.Y., First ed., 1951, pp. 5 and 10.